

## UNITED STATES PATENT OFFICE

ERICH WIEGAND, OF BERLIN-WAIDMANNSLUST, GERMANY, ASSIGNOR TO GENERAL ELECTRIC COMPANY, A CORPORATION OF NEW YORK

## MANUFACTURE OF HOT CATHODES FOR ELECTRIC DISCHARGE DEVICES

No Drawing. Application filed February 11, 1932, Serial No. 592,450, and in Germany February 14, 1931.

The present invention relates to hot cathodes for electric discharge devices. One of the objects of the invention is to provide a process for the production of a homogeneous 5 alkaline earth alloy suitable for use as a hot cathode in electric discharge devices. A further object of the invention is to provide a cathode structure having a high emission capacity and a relatively long life. Other 10 objects will appear hereinafter.

Heretofore it has been proposed to employ metals of the alkaline earth group, particularly barium, directly as emission bodies. Since barium melts at about 650° C. and also 15 vaporizes very easily it can be employed only in the form of a coating on metals of high melting point or as an alloy with such metals. Thus it is known, for example, that metals, like platinum, that form alloys with barium, 20 can be superficially alloyed with barium by heating in barium vapor, and, in some cases after oxidizing a part of the barium metal contained in the alloy, these bodies may be employed as cathodes. Cathodes produced 25 in this way have, however, the disadvantage that the alkaline earth metal content is consumed comparatively quickly as generally only a thin superficial layer contains the active metal.

Efforts to produce a homogeneous alkaline earth alloy useful for hot cathodes have heretofore been unsuccessful. This has been due partly to the fact that melts of the two 30 constituents can be produced only with great difficulty since barium metal vaporizes very easily. Also it has been found that it is not possible to obtain a homogeneous alloy by causing barium metal in the form of a liquid 35 or a vapor to act on solid bodies of metals of high melting point, because the alkaline earth metal penetrates only very slowly into the deeper layers.

I have discovered that barium metal in a molten condition wets metallic bodies extremely readily and use is made of this 40 property in the production of alkaline earth alloys according to the present invention. If one treats with molten barium a porous metal body such as may be very easily produced by 45 pressing metal powder in suitable apparatus,

the barium very quickly fills the pores completely. The alkaline earth metal and the metal of high melting point are thus well mixed together and by suitable heat treatment this mixture can be easily transformed 55 into a homogeneous alloy.

For many purposes it is not necessary to transform the whole of the barium metal present in the metal body into the alloy. Even a small formation of alloy is sufficient 60 to prevent the escape of the barium metal during the further treatment and to produce useful cathodes.

The barium content of the alloy produced according to the new process is generally determined by the volume of the pores of the 65 body of the metal of high melting point. By a sintering treatment of the metal body before the alloying action, the volume of the pores can be altered considerably, and in this 70 way alloys with different alkaline earth content can be prepared without difficulty.

The alloyed rods can be worked up in a known manner into wire-shaped or strip-shaped cathodes. In doing this it is desirable to anneal the impregnated metal bodies 75 from time to time in a vacuum or in a rare gas atmosphere. Such cathodes can be made without difficulty from, for example, alloys of barium with nickel or platinum having a 80 barium content up to about 10%. Alloys with still higher barium content can be prepared mechanically but only with difficulty.

The present process can be applied also with advantage in producing in a simple 85 manner very uniform mixtures of barium with metals that do not form alloys therewith, as tungsten, molybdenum, tantalum, etc. Such metal bodies, if their barium content is not too great may be worked up me- 90 chanically without difficulty and employed for cathodic purposes with good results. Finally, instead of pure barium, easily fusible alloys, as barium-aluminum, barium copper, etc. can be caused to act on the porous metal 95 bodies and the electrical and mechanical properties of the metal bodies can thus be considerably improved.

For many purposes it is advantageous to treat the porous metal bodies in a stream of 100

alkaline earth metal vapor rather than with molten metal. When thus treated, alloys with more than 5% of barium generally cannot be produced. However, alloys prepared in this way are characterized by great purity. As by far the greatest proportion of barium compounds are less fusible than barium, in this process only pure barium can enter into the metal bodies.

10. Cathodes prepared according to the described process can be employed either directly in discharge tubes with or without gas filling or after they have been coated in known manner with alkaline earth oxides.

15. The cathodes are distinguished by a high emission capacity and long duration.

What I claim as new and desire to secure by Letters Patent of the United States, is:

20. 1. The process of producing a metallic structure suitable for use as a hot cathode which comprises pressing a powdered metal of high melting point thereby to provide a porous body and impregnating said body with molten material comprising an alkaline earth metal.

25. 2. The process of producing a metallic structure suitable for use as a hot cathode which comprises pressing a powdered metal of high melting point thereby to provide a porous body and impregnating said body with molten barium.

30. 3. The process of producing a metallic structure suitable for use as a hot cathode which comprises pressing powdered nickel into a desired shape to thereby provide a porous body and impregnating said porous body with molten barium.

35. 4. The process of producing a metallic structure suitable for use as a hot cathode which comprises pressing a powdered metal of high melting point thereby to provide a porous body, impregnating said porous body with molten material comprising an alkaline earth metal and heating said impregnated body thereby to form an alloy of said metal with at least a portion of said alkaline earth metal.

40. 5. The process of producing a metallic structure suitable for use as a hot cathode which comprises pressing a powdered metal of high melting point in a mold, impregnating said powdered metal with molten barium, mechanically working the impregnated body into a desired shape and annealing said impregnated body at intervals during the working process.

45. 6. The process of producing a metallic structure suitable for use as a hot cathode which comprises pressing powdered, high melting point metal in a mold, partially sintering said pressed material to thereby control its porosity, impregnating said partially sintered material with a molten alkaline earth metal, mechanically working the impregnated body into a desired shape and an-

nealing said impregnated body at intervals during the working process.

In witness whereof, I have hereunto set my hand.

ERICH WIEGAND.

70

75

80

85

90

95

100

105

110

115

120

125

130